

# UNITED STATES PATENT OFFICE.

CHARLES OWEN GRIFFITH, OF ROCKVILLE, WORMIT, SCOTLAND.

## PROCESS FOR THE PRODUCTION OF METALLIC SULFIDS.

1,261,023.

Specification of Letters Patent. Patented Apr. 2, 1918.

No Drawing.

Application filed June 7, 1917. Serial No. 173,309.

*To all whom it may concern:*

Be it known that I, CHARLES OWEN GRIFFITH, citizen of Great Britain, and resident of Rockville, Wormit, in the county of Fife, Scotland, have invented certain new and useful Improvements in Connection with Processes for the Production of Metallic Sulfids, of which the following is a specification.

10 This invention relates to the production of metallic sulfids and has for its object to provide a process whereby sulfids of metals may be produced by an electrical process.

According to this invention, I employ a 15 cell in which is placed a metal plate or the like forming the anode, the cathode being formed by a plate or the like of the same metal coated or incrusted in whole or in part, with sulfur.

20 In one manner of carrying out my process I employ a zinc anode of round, flat, or other suitable section and a cathode formed of a stick or plate of zinc covered with sulfur. As an electrolyte I use a solution of 25 ammonium chlorid or other suitable chlorid with or without the addition of other agents. To the anode I connect the positive conductor of a generator or other source of current and to the cathode I connect the negative conductor. Upon the current passing 30 through the cell sulfureted hydrogen appears to be given off at the cathode, and zinc sulfid is deposited in the cell, from whence it may be collected and treated so as to 35 eliminate any impurities.

The chief difficulties attending the manufacture of metallic sulfids by electrolysis are connected with the elimination or avoidance of impurities and my process goes further 40 in attaining this object than any I know of, because the anode and cathode are the only metal introduced into the cell and they are formed of the metal of which it is desired to obtain the sulfid. My preferred manner 45 of applying the cathode covering of sulfur, is performed as follows:—A shallow crucible of convenient size, or a vessel made of the clay or earth from which crucibles are mostly made, is used in melting the sulfur 50 in preference to an iron or tin plate vessel, which if heated without extreme care causes impurities to be formed, besides which the vessel becomes very quickly useless by oxidation. I use the best quality of rock sulfur, 55 and, when heat is applied until it has melted, I then place the metal plate to be coated

face downward touching the molten sulfur for a few moments, it afterward being withdrawn and allowed to cool. It is then dipped again and the operation repeated 60 until a coating of the desired thickness has been obtained. It depends upon the strength of current used how much of the plate should be coated. In my original experiment the only current available was a 65 very strong one and the plate, which was about 3 inches in area,  $1\frac{1}{2}$  inches thick, was only partly covered with sulfur about  $\frac{1}{4}$  thick. The result was that along with the sulfid formed there were metallic deposits 70 from the anode which were difficult to remove.

By coating the rest of the plate with a thin film of sulfur I found that the sulfid was produced free of metallic deposit. By 75 a careful regulation of the current, however, and keeping it constantly below  $1\frac{1}{2}$  volts and 4 amperes at a temperature of 50° C. to 70° C. and at or above 1 volt and 2 amperes, I found it necessary to coat only 80 part of the plate either in the manner above described or by pouring the melted sulfur into a mold and placing the block thus formed (after dipping it into the melted sulfur) upon the metal. When only part 85 of the metal is coated it does not appear to make much difference how thick the block is, provided it is maintained in position. I prefer this latter method, as the sulfur lasts longer and as the electrolyte seldom requires to be renewed. 90

Temperature, strength of current and method of coating are important in obtaining the best colors of the various sulfids. The figures I have given apply particularly 95 well in the case of antimony, and generally speaking to all the other sulfids. Should these conditions not be strictly observed, particularly in the case of antimony  $H_2S$  is given off in an offensive quantity and there 100 are impurities which affect the color adversely.

To produce other metallic sulfids a similar process is employed, except that the zinc anode and cathode are substituted by an 105 anode and cathode of the metal of which it is desired to obtain the sulfid.

It may also be necessary or desirable to vary the electrolyte to suit the particular metal employed in the process.

110 I have mentioned the employment of ammonium-chlorid as an electrolyte in connec-

tion with the production of sulfid of zinc, but I may find that some other agent might be more suitable.

For instance as an electrolyte, in the case of antimony, I use sodium chlorid, ammonium chlorid or antimony trichlorid, and in the case of zinc, iron, lead, copper, cadmium, silver, arsenic and mercury, sodium chlorid, or ammonium chlorid, may be used.

10 I have also tried the chlorid of the metal of which it is desired to obtain the sulfid and this appears to do quite well either alone or in conjunction with sodium chlorid or ammonium chlorid.

15 I claim:—

1. A process for the production of metallic sulfids consisting of passing an electrical current through a cell provided with an electrolyte and in which the anode and cath-

ode are formed of the same kind of metal, 20 the cathode being provided with sulfur.

2. A process for the production of sulfid of zinc in which the anode and cathode are of zinc and are immersed in a chlorid, the cathode being provided with sulfur.

25 3. A process for the production of sulfid of zinc in which the anode and cathode are formed of zinc and are immersed in a chlorid, the cathode being partly coated with sulfur.

Signed at Dundee, in the county of Forfar, Scotland, this sixteenth day of May, A. D. 1917.

CHARLES OWEN GRIFFITH.

Witnesses:

JESSIE MORTON,  
THEODORE WILLIAM DRUBBLE.